

July 18, 1950

E. R. BOLLER ET AL

2,515,488

PROCESS OF CLEANING AND COATING FERROUS METAL

Filed March 12, 1946



INVENTORS  
*Ernest R. Boller,  
Lowell D. Eubank &  
Clarence A. Littler  
BY Fred C. Carlson*

ATTORNEY

Patented July 18, 1950

2,515,488

# UNITED STATES PATENT OFFICE

2,515,488

## PROCESS OF CLEANING AND COATING FERROUS METAL

Ernest R. Boller, Marion, Ind., and Lowell D. Eubank, South Euclid, and Clarence A. Littler, Maple Heights, Ohio, assignors to E. I. du Pont de Nemours & Company, Wilmington, Del., a corporation of Delaware

Application March 12, 1946, Serial No. 653,968

5 Claims. (Cl. 117—51)

1

This invention relates to the coating of ferrous articles with a zinc aluminum alloy and is more particularly directed to processes in which a ferrous article is first passed through a molten zinc chloride flux which is supported upon a mass of molten zinc and thereafter passed through a molten zinc-aluminum alloy containing less than about 0.05 per cent by weight of iron.

Methods for galvanizing, in which ferrous articles are passed through a molten flux layer supported upon a bath of molten zinc and then through the zinc, are well understood, but when it is attempted to adapt such galvanizing techniques to methods for coating ferrous articles with molten zinc-aluminum alloys difficulties are immediately encountered. First, fluxing techniques for cleaning the metal are found to be inadequate. When zinc chloride-ammonium chloride fluxes are used on top of the molten alloy it is found that the flux rapidly becomes so viscous that it soon loses its cleaning and fluxing ability and becomes impossible to use. Moreover when procedures ordinarily used in zinc galvanizing are applied to zinc-aluminum galvanizing it is found that the molten alloy becomes badly contaminated with dross and that the alloy coating on the articles as withdrawn from the molten metal is marred by dross. These difficulties are encountered even when the aluminum content of the bath is as low as from  $\frac{1}{2}$  to  $1\frac{1}{2}\%$ . That so small an aluminum content should give rise to such pronounced difficulties is surprising but nevertheless is the fact and the lack of a solution to these problems has mitigated against the widespread production of zinc-aluminum coatings even though it was recognized that such coatings have better tightness and corrosion resistance than ordinary zinc coatings.

It is an object of this invention to provide galvanizing processes which are simple and economical and which yield coated ferrous articles of good appearance and character. It is a further object to provide adherent coatings of zinc-aluminum alloys upon ferrous articles. It is a still further object to provide a process for cleaning steel prior to coating with a zinc-aluminum alloy. Further objects will become apparent hereinafter.

Described with reference to the drawing, the foregoing and other objects of the invention are attained by first passing a ferrous article, 1, through a molten zinc chloride flux, 2, which is supported upon a bath of molten zinc, 3. The ferrous article is then removed from the flux, without its being permitted to come in contact with the zinc, and is passed into a zinc-aluminum galvanizing bath, 4, containing not more than about 0.05 per cent by weight of iron.

By use of the processes of the invention one is enabled economically and practically to use zinc-

2

aluminum alloys for the coating of steel and other ferrous articles. The articles are readily cleaned at low cost without the use of expensive cleaning agents or processes such as those involving inert atmospheres and without rapid destruction of the main flux body.

The flux bath employed according to the present invention is comprised of molten zinc chloride. This may additionally contain ammonium chloride or zinc ammonium chloride which will in the course of use be converted to zinc chloride by the underlying molten zinc layer. Other flux salts and additions may be included as desired. While the molten zinc chloride should be the principal constituent, the flux in a preferred embodiment of the invention desirably may contain an alkali metal chloride, or a mixture of alkali metal chlorides such as sodium chloride and potassium chloride, in an amount up to about 25 per cent by weight. A mixture of 95% commercial zinc chloride, 2.5% sodium chloride, and 2.5% potassium chloride has given excellent results.

This molten flux is supported upon molten zinc. The zinc functions to remove iron compounds from the flux and continuously prevents "build-up" of iron compounds in the flux. The amount of molten zinc must be sufficient with relation to the amount of flux to maintain continuously a sufficiently low iron content. The rate of iron removal in a well agitated bath with a fixed Zn area is a function of the concentration of iron in the flux which, for instance, with 42# flux and a Zn surface of 0.441 sq. ft. can be expressed by the empirical relationship:

$$t = -3.98 - 6.17 \log C$$

where  $t$  = time (hours) and  $C$  = iron content (%). From this equation the rate of iron removal

$$\frac{dc}{dt}$$

at any iron concentration can be determined.

For example the removal rate at 0.1% Fe was 0.0352 lbs. Fe per hour per sq. ft. of zinc surface.

It will also be understood in this connection that the rate of passage of ferrous articles through the flux must not be too slow nor the total surface passed per unit of time too fast with relation to the amount of zinc and the amount of flux or the iron "build-up" may exceed the rate of removal by the zinc. Iron dissolved in the flux from the ferrous articles, and if the articles remain too long in the flux, the iron dissolves to an undesirable degree. An idea of the rate of such dissolution may be gained from the fact that, in a flux containing 95% commercial zinc chloride, 2.5% sodium chloride, and 2.5% potassium chloride at  $450^\circ$  C.,  $2.05 \times 10^{-4}$  lbs. of steel

3

per sq. ft. of surface of 24 gage steel sheet was dissolved during a five second exposure.

The iron removed from the flux forms as a dross in the zinc metal and, being more dense than the zinc, sinks to the bottom. This is shown as 5 in the drawing.

The zinc used for the molten sub-stratum may be composed of any of the ordinary commercial grades of zinc such as Special Hi grades, Intermediate, Selected or Prime Western.

The zinc-aluminum alloy constituting the galvanizing bath should contain at least about 0.2% of aluminum, and it is particularly preferred that the bath contain from about 0.2% to 1.5% of aluminum. As in the case of the sub-stratum above described, the zinc used for the galvanizing bath may be any of the commercial grades of zinc. Electrolytic zinc would be preferred except for its somewhat higher cost. "Selected" zinc or "Prime Western" zinc may be used, the latter however, only if the Fe content is below the maximum allowable 0.08% or if it be mixed with a suitable quantity of Zn low in Fe. It is therefore ordinarily desirable to select a zinc with as low an iron content as practicable say of the order such that total iron during continuous running does not build up to exceed about 0.05%.

The galvanizing bath may of course contain minor additions such as tin, lead, antimony, or cadmium in accordance with standard practices although these are not generally preferred. In any event it will ordinarily be preferred that the zinc content of the galvanizing bath exceed about, say, 98%.

It will be understood that iron dissolves from the ferrous objects being coated in the zinc-aluminum bath, and therefore the time of contact of the objects with the zinc-aluminum should be as short as feasible. In a particular case, for example, the rate of dissolution of iron from 24 gage cold-rolled sheet in a 99.5% zinc-0.5% aluminum bath was found to be  $9.07 \times 10^{-6}$  lbs. per sq. ft. of surface for a 5 second dip.

It will be seen that by the operation of a process as above described one is enabled quickly, economically, and efficiently to clean ferrous articles prior to galvanizing and to provide ferrous articles which contain little or no iron compounds on their surfaces. This is important for the presence of such compounds as has heretofore been indicated rapidly causes deterioration of a zinc-aluminum galvanizing bath by forming objectionable dross.

The invention may be better understood by reference to the following illustrative example:

*Example*

A quantity of 24 gage cold-rolled steel is prepared for treating according to a process of this invention by pickling for five minutes in 9% sulfuric acid aqueous solution inhibited with 0.05% of sulfurized quinoidine at 80° C., for 30 seconds in hot water, dipped for one minute in a solution of 0.1% tetrasodium pyrophosphate-0.1% soap solution at 80° C. and rinsed again in hot water for 30 seconds.

The sheet, so prepared, is dipped while still wet and hot into a molten flux comprising 95% commercial zinc chloride, 2.5% sodium chloride, and 2.5% potassium chloride maintained at 450° C. over a substratum of molten zinc with which the steel makes no contact.

After 5 seconds in the molten flux, during

4

which the sheet was completely cleaned of iron salts and oxides, the sheet was withdrawn, rapidly scraped free of all but a thin film of flux, and dipped while hot in a bath of molten zinc-aluminum comprising 99.5% Grasselli Select zinc and 0.5% aluminum at 430° C. The sheet is withdrawn in 5 seconds and excess coating removed by shaking. The resultant coating is free of visible dross crystals and is exceedingly adherent as determined by tests of direct adhesion and by flexing tests where the steel could be ruptured without flaking off the zinc-aluminum coating.

We claim:

15. 1. In a process for galvanizing the steps comprising supporting a molten zinc chloride layer upon and in contact with a molten zinc bath, passing a ferrous article into and out of said supported zinc chloride layer only, and then passing the ferrous article while still hot through a molten zinc-aluminum bath which does not contain more than about .05% of iron.

2. In a process for applying a zinc-aluminum coating to a ferrous article the steps comprising supporting a molten zinc chloride layer upon and in contact with a molten zinc bath, passing a ferrous article into and out of said supported zinc chloride layer only, and then passing the ferrous article while still hot through a molten zinc-aluminum bath which contains 0.2 to 1.5% aluminum and which does not contain more than about 0.05% of iron.

3. In a process for applying a zinc-aluminum coating to a ferrous article the steps comprising supporting a molten zinc chloride layer containing an alkali metal chloride upon and in contact with a molten zinc bath, passing a ferrous article into and out of said supported zinc chloride layer only, and then passing the ferrous article while still hot through a molten zinc-aluminum bath which contains 0.2 to 1.5% aluminum and which does not contain more than about 0.05% of iron.

4. In a process for cleaning a ferrous metal the steps comprising supporting a molten zinc chloride layer upon and in contact with a molten zinc bath, and passing the ferrous metal into and out of said supported zinc chloride layer only.

5. In a process for cleaning a ferrous metal the steps comprising supporting a molten zinc chloride layer containing an alkali metal chloride upon and in contact with a molten zinc bath, and passing the ferrous metal into and out of said supported zinc chloride layer only.

ERNEST R. BOLLER.  
LOWELL D. EUBANK.  
CLARENCE A. LITTLER.

REFERENCES CITED

The following references are of record in the file of this patent:

UNITED STATES PATENTS

| Number    | Name      | Date          |
|-----------|-----------|---------------|
| 244,153   | Spear     | July 12, 1881 |
| 1,276,977 | Shoemaker | Aug. 27, 1918 |
| 1,334,092 | Harmeling | Mar. 16, 1920 |
| 1,374,233 | Reinhold  | Apr. 12, 1921 |
| 1,722,949 | Wehr      | July 30, 1929 |
| 1,741,388 | Wehr      | Dec. 31, 1929 |
| 1,965,759 | Baldwin   | July 10, 1934 |
| 2,008,879 | Simmons   | July 23, 1935 |
| 2,095,198 | Reid      | Oct. 5, 1937  |
| 2,101,553 | Mattsson  | Dec. 7, 1937  |